

**[54] PROCESS FOR PRODUCING HARD MAGNETIC MATERIAL**

[56]

**References Cited****U.S. PATENT DOCUMENTS**

1,986,197 1/1935 Harshaw ..... 75/212

**FOREIGN PATENT DOCUMENTS**

566352 11/1958 Canada ..... 75/212

51-21947 of 0000 Japan .

811935 4/1959 United Kingdom ..... 75/212

779969 7/1957 United Kingdom ..... 75/212

**[75] Inventors:** Takeo Sata; Masayuki Takamura; Toshiharu Hoshi, all of Hamamatsu, Japan**[73] Assignee:** Nippon Gakki Seizo Kabushiki Kaisha, Japan**[21] Appl. No.:** 226,923**[22] Filed:** **Jan. 21, 1981****[30] Foreign Application Priority Data**

Jan. 24, 1980 [JP] Japan ..... 55-6369

**[51] Int. Cl.<sup>3</sup>** ..... **B22F 1/02****[52] U.S. Cl.** ..... **419/23; 419/28;**  
**419/26; 419/35; 148/120****[58] Field of Search** ..... **75/212, 214, 29/420.5;**  
**264/176 R, 320, 325; 148/104, 105, 120;**  
**419/23, 28, 26, 35***Primary Examiner*—Jack Cooper*Attorney, Agent, or Firm*—Lerner, David, Littenberg, Krumholz & Mentlik

[57]

**ABSTRACT**

In production of so-called anisotropic fine gain type hard magnetic material, particles of highly magnetic substance powder are each plated with nonmagnetic substance before compaction, sintering and plastic deformation in order to provide the product with stable magnetic characteristics for reduced production cost.

**4 Claims, 9 Drawing Figures**

PRIOR ART

Fig. 1A



PRIOR ART

Fig. 1B



PRIOR ART

Fig. 2



Fig. 3



Fig. 4





Fig. 5



Fig. 6



Fig. 7



Fig. 8

PROCESS FOR PRODUCING HARD MAGNETIC MATERIAL

BACKGROUND OF THE INVENTION

The present invention relates to a process for producing hard magnetic material, and more particularly relates to a process for producing so-called anisotropic fine grain type hard magnetic material in which fine grains each corresponding to a unit magnetic domain are dispersed with shape anisotropy into a nonmagnetic base.

It is well known to public to produce hard magnetic material with magnetic anisotropy and high magnetic characteristics by dispersing with prescribed orientation into a base of nonmagnetic substance such as Cu, Al and Sn anisotropic fine grains of highly magnetic or ferromagnetic substance such as Fe, Co, Ni and Fe-Co alloys, each grain corresponding to a unit magnetic domain.

In one actual process for production of such hard magnetic material, cast Fe-Ni-Al-Co type alloy, or like alloy further including Cu, Ti and/or Nb, is thermally treated within magnetic field in order to cause so-called spinodal decomposition which eventuates in dispersed separation of highly magnetic, fine grains with shape anisotropy within a nonmagnetic phase. This process, however, results in high material cost due to use of costly metals such as Co and Ni. In addition, the thermal treatment within magnetic field requires use of an exorbitant equipment, and causes high process cost and low productivity. Further, the hard magnetic material produced by this process is too hard and fragile to be worked and/or cut smoothly.

In another actual process for production of the above-described hard magnetic material, fine, spherical Fe grains, each having a diameter in a range from 15 to 30 mm and corresponding to a unit magnetic domain, are obtained by a reduction process. Such Fe grains are then blended with grains of nonmagnetic metal such as Al, and the resultant blend is subsequently subjected to compaction and sintering.

In the case of this process, however, it is extremely infeasible to prepare fine grains of uniform diameter, each corresponding to a unit magnetic domain, since such fine grains easily aggregate even in a free state due to mutual magnetic attraction. Relatively large specific surface area of each fine grain tends to cause oxidization of the grains, which disables easy and simple handling of the substance. Oxidization of the substance seriously degrades saturated magnetic flux density  $B_s$  and  $4\pi M_s$  of the resultant, sintered material. Such oxidization further impairs affinity of the grains with the grains of nonmagnetic substance, thereby seriously deteriorating mechanical strength of the obtained sintered body. Ill spinal rotation due to presence of the spherical grains is liable to connect to unstable magnetic characteristics of the product.

In the other actual process of the above-described hard magnetic material, long and thin Fe fine grains or Fe-Co alloy fine grains are separated on Hg electrodes by electrolysis which are then dispersed into nonmagnetic substance, the blend is processed to compaction for orientation of the Fe fine grains, and the compacted body is subjected to sintering. Although this process significantly improves magnetic characteristics of the product, it is still very difficult to obtain, at high efficiency, fine grains of uniform dimension. Further, this

process, just like the foregoing instance, cannot avoid the oxidization troubles.

It is also proposed in actual production of the hard magnetic material of the above-described type to subject a highly magnetic core rod, e.g. an Fe rod, covered with a nonmagnetic sheath, e.g. an Al sheath, to repeated drawings for plastic deformation, which microminiaturizes and disintegrates the highly magnetic substance into mutually separated fine grains, each corresponding to a unit magnetic domain, dispersed within the nonmagnetic base.

In this case, however, high frictional contact between the highly magnetic core covered with the nonmagnetic sheath and the dies disables uniform flow of the substances during the process. Consequently, the highly magnetic fine grains are oriented substantially in parallel to the axial direction of the product in its central section whereas they are arranged at random in the peripheral section of the product. Such untidy arrangement of the highly magnetic fine grains within the obtained structure seriously deteriorates magnetic characteristics of the resultant hard magnetic material. Since it is difficult to design a high rate of cross-sectional reduction for each drawing, drawings have to be repeated several times in order to obtain a product of a desired diameter, thereby considerably raising production cost.

A process for solving such problems has already been proposed by inventors of the present invention in Japanese Publication Sho. No. 51-21947, in which the conventional drawing process is replaced by hydrostatic extrusion process for production of a hard magnetic material. This proposal is based on a recognition that relatively low frictional contact between the work piece and the die allows smooth and tidy flow of the substances and relatively high rate of cross-sectional reduction is employable in the case of the hydrostatic extrusion. In this proposed process, a plurality of elongated highly magnetic cores each covered by nonmagnetic sheath are bundled together and subjected to hydrostatic extrusion for plastic deformation. As a result of such plastic deformation, highly magnetic fine grains, each corresponding to a unit magnetic domain, are oriented and dispersed within the nonmagnetic base so that their longitudinal directions substantially meet the axial direction of the produced hard magnetic material which has a composit structure with shape anisotropy.

This process assures ideal orientation of the fine grains, each corresponding to a unit magnetic domain and, consequently, greatly improved magnetic characteristics of the product. Production requires reduced repetition of the unit operation, i.e. the hydrostatic extrusions, thereby remarkably lowering the production cost.

Further study of this previous process by the inventors, however, has revealed presence of the following disadvantage. As described already, the highly magnetic core, e.g. an Fe rod, is covered with the nonmagnetic sheath such as Al covering in the case of this previously proposed process, prior to the hydrostatic extrusion. More specifically, a Fe rod is inserted into a small Al cylinder, whose inner wall is covered with  $\text{Al}_2\text{O}_3$  layer, in order to form a composite body. A plurality of such composite bodies are bundled together, inserted into a large Al cylinder and subjected to hydrostatic extrusion for cross-sectional reduction of the composite bodies.

Since each Fe rod is broken into fine pieces during the plastic deformation, cross-sectional reduction tends to vary from piece to piece. Consequently, the Al base of the product contains Fe fine grains of different diameters. Some fine grains may be larger in size than the unit magnetic domain, and uncontrollable presence of such large fine grains dispersed in the base leads to unstable magnetic characteristics of the obtained hard magnetic material. With this previous process, it is almost infeasible to control the hydrostatic extrusion so that the product should contain Fe fine grains only which correspond in size to the unit magnetic domain. When compared to the conventional production by rawing, use of hydrostatic extrusion remarkably reduces repetition of the unit operation thanks to its relatively large extrusion ratio. Yet, appreciable repetition of the hydrostatic extrusion is necessary to miniaturize the starting rod to the fine grains each corresponding to a unit magnetic domain. Employment of high rate cross-sectional reduction for hydrostatic extrusion in this process may limit free choice of the substances to be used due to expected high resistance against plastic deformation.

#### SUMMARY OF THE INVENTION

It is one object of the present invention to produce a hard magnetic material with stable magnetic characteristics.

It is another object of the present invention to produce a hard magnetic material by hydrostatic extrusion with appreciably reduced production cost when compared with the previously proposed process by hydrostatic extrusion.

It is the other object of the present invention to produce a hard magnetic material whilst successfully obviating malignant influence of oxidation which is inherent in the conventional process by powder metallurgy.

In accordance with the basic aspect of the present invention, particles of highly magnetic substance powder are each plated with nonmagnetic substance in advance to compaction, sintering and plastic deformation in a prescribed direction so that fine grains of the highly magnetic substance are dispersed with shape anisotropy into the base of the nonmagnetic substance.

#### BRIEF DESCRIPTION OF THE DRAWINGS

FIG. 1A is a perspective view of the composite body used for the process previously proposed by the inventors of the present invention.

FIG. 1B is an end view of the composite bodies of FIG. 1 assembled together for hydrostatic deformation.

FIG. 2 is a cross-sectional model view of the hard magnetic material produced by the process previously proposed by the inventors.

FIG. 3 is an end view of the sintered bodies obtained in the process of the present invention.

FIG. 4 is a cross-sectional model view of a hard magnetic material in accordance with the present invention, and

FIGS. 5 through 8 are graphs for showing magnetic characteristics of the obtained hard magnetic material for various combinations of Fe with nonmagnetic metals.

#### DESCRIPTION OF THE PREFERRED EMBODIMENTS

As briefly described already, the process previously proposed by the inventors of the present invention uses,

as the starting material, a composite body 4 such as shown in FIG. 1A, and a plurality of such composite bodies 4 are bundled together and inserted into a large cylinder 6 as shown in FIG. 1B for plastic deformation by hydrostatic extrusion. The composite body 4 may include an Al cylinder 3 internally coated with an Al<sub>2</sub>O<sub>3</sub> layer 2 and an Fe rod 1 inserted into the Al cylinder 3.

Internal structure of a hard magnetic material produced by the above-described process is illustrated in FIG. 2, in which Fe fine grains 1a of various diameters R1, R2 and R3 are dispersed in an Al base 3a. Some Fe fine grains are larger in size than the unit magnetic domain and their presence in the structure seriously degrades stability in magnetic characteristics of the obtained hard magnetic material.

As a result of repeated study, it was confirmed by the inventors of the present invention that difficulty in cross-sectional reduction to the level of the unit magnetic domain is caused by occurrence of slip at the border between Fe and Al during the plastic deformation which seriously bars uniform application of the deformative force from the die to the Fe component.

In order to prevent such slip, it is effective first to miniaturize highly magnetic substance such as Fe to powder particles to an extent larger than the unit magnetic domain and plate such powder particles with nonmagnetic substance such as Cu. Such plated particles are then subjected to plastic deformation in a prescribed direction after compaction and sintering so that the highly magnetic powder particles are elongated in the direction at uniform rate of cross-sectional direction without any slip at the border between the two substances.

Metals such as Fe, Co, Ni and alloys including two or more of them are advantageously used for the highly magnetic or ferromagnetic substance in the process of the present invention, and metals such as Cu, Al Sn, Pb, Zn and combination of these metals are advantageously used for the nonmagnetic substance. Combination of these substances should be small in solid solution limit so that no separate phase should be developed in sintering due to excessive dispersion at the border between the highly magnetic and nonmagnetic substances. For example, combination of Fe with Cu is ideal.

It was experimentally confirmed that combinations of ferromagnetic and nonmagnetic substance such as shown in the following table brought about highly improved magnetic characteristics of the product as shown in FIGS. 5 through 8.

| Combination | Volume occupation ratio of Fe in % |
|-------------|------------------------------------|
| Fe/Cu       | 10 to 85                           |
| Fe/Pb       | 10 to 85                           |
| Fe/Sn       | 10 to 80                           |
| Fe/Zn       | 10 to 80                           |

Here, the term "Volume occupation ratio of Fe" refers to percent volume content of Fe in the volume of the combination.

Preparation of the starting highly magnetic powder particles is carried out in various known ways such as carbonyl powder production methods and atomization methods. In order to successfully obtain final grains each corresponding to a unit magnetic domain, it is advantageous to prepare powder particles of substantially similar diameters by proper filtering.

The particle diameter should preferably in a range from 1 to 1,000  $\mu\text{m}$ , and more favourably from 5 to 150  $\mu\text{m}$ . Any particle diameter smaller than 1  $\mu\text{m}$  tends to cause aggregation of the powder particles which seriously hinders preparation of particles of uniform diameter by the filtering. Such small particle size also causes easy oxidization of the highly magnetic substance, thereby impairing the magnetic characteristics of the product. Whereas any particle diameter larger than 1,000  $\mu\text{m}$  calls for increased repetition of the treatment necessary for microminiaturization to the unit magnetic domain level, thereby increasing the production cost. During the subsequent plastic deformation, cross-sectional reduction elongates each powder particle in the direction of orientation in order to improve its magnetic characteristics. But, since this effect saturates beyond the particle diameter of 1,000  $\mu\text{m}$ , there is no significance in further enlarging the particle diameter.

Although it is usual to use highly magnetic powder particles of spherical shapes, particles like short fibers may be used depending on the situation.

The highly magnetic powder particles are plated with the nonmagnetic substance by, for example, non-electrolytic plating. More specifically, when Fe is used for the highly magnetic substance and Cu is used for the nonmagnetic substance, Fe powder particles are added to copper salt solution such as copper sulfate solution which contains about 0.5 to 100 g/l of copper and 0.05 to 10% of sulfuric acid as a reaction accelerator. Then Fe particles are plated with Cu due to the following substitution reaction.



In this case, the quantity of the Fe particles to be added is about 20 times of the chemical equivalent necessary for the substitution. Next, the Cu plated particles are subjected to appropriate cleansing and drying. When required, they may be subjected to reduction within a reducing gas environment such as  $\text{H}_2$  gas.

After the above-described plating with nonmagnetic substance such as Cu, the plated Fe particles are subjected to compaction such as hydrostatic extrusion, and further to sintering within a non-oxidizable environment such as  $\text{H}_2$  gas. Process conditions for this sintering differ depending on the type of combination of the starting substances. In the case of Fe particles plated with Cu, sintering is preferably carried out at a temperature in a range from 450° to 950° C. for 0.5 to 5 hours. The cross-sectional structure of the resultant sintered body is shown in FIG. 3, in which Fe fine grains 7 are wholly covered with Cu plates 8.

Next, the sintered body is subjected to plastic deformation in a prescribed direction such as hydrostatic extrusion. After the deformation, the material has a structure shown in FIG. 4, in which highly magnetic fine grains 7a of substantially uniform diameter R are dispersed and oriented within a nonmagnetic base 8a whilst extending in the direction of extrusion A.

This plastic deformation may be carried out by extrusion other than hydrostatic or drawing also either in hot or cold state. Hydrostatic extrusion, however, is advantageous since it allows employment of large extrusion ratios. In addition, extremely low frictional contact between the die and the sintered work piece allows, even in the peripheral section of the work piece, flow of the substances in parallel to the axis of the work piece, which eventuates in tidy and uniform orientation of the highly magnetic fine grains, thereby assuring improved

magnetic characteristics of the resultant hard magnetic material.

The above-described plastic deformation should be carried out until the diameter of the highly magnetic fine grains eventually corresponds to that of a unit magnetic domain. Therefore, extrusion rate for each plastic deformation and the number of repetition of the plastic deformation are designed in reference to the initial particle size. Annealing is usually applied to the work piece after each plastic deformation. It is also usual that, after a certain plastic deformation is over, a plurality of work pieces reduced in diameter in that plastic deformation are bundled together for a next plastic deformation. Here, the size of the unit magnetic domain, i.e. the critical radius, differs depending on the kind of the highly magnetic substance. It is roughly 8 to 15 mm. for Fe, 3 mm. for Co and 27 mm. for Ni.

Since the nonmagnetic substance used for the plating is very strongly bonded to the highly magnetic powder particles, no slip occurs at the border between the two substances during plastic deformation. Consequently external force acting on the sintered body is uniformly and sufficiently transmitted to the highly magnetic particles so that the particles can be well deformed monolithically with the nonmagnetic substance plated on them. As a result, the highly magnetic powder particle can be microminiaturized uniformly whilst being wholly covered with the nonmagnetic base. It is believed also that the total covering of the highly magnetic particles with the nonmagnetic substance well contributes to absence of slip at the border between the two. For these reasons, the above-described monolithic deformation occurs even when the nonmagnetic substance is poorer in deformation resistance than the highly magnetic particles it covers.

The exquisitely microminiturized and oriented arrangement of the highly magnetic fine grains within the nonmagnetic base assures high coercive force  $H_c$ , residual magnetic flux density  $B_r$  and maximum magnetic energy product  $(BH)_{max}$  of the produced hard magnetic material.

In accordance with the process of the present invention, the highly magnetic metal used for the starting substance is already powdered to an appreciable particle size and such advanced minituarization of the starting substance greatly reduces the number of repetitions of the subsequent plastic deformation necessary for further microminiaturization to the unit magnetic domain level when compared with the above-described previously proposed process. In other words, it is no longer required to employ a large deformation ratio for each plastic deformation and, therefore, choice of substance is no longer restricted by deformability of the substance.

Further, presence of the subsequent microminiaturization allows use of a starting substance of a particle size significantly larger than that of the unit magnetic domain. This enables easy preparation of the highly magnetic substance, and ideal filtering of the highly magnetic powder particles. The large particle size also precludes, or to say the least diminishes, the oxidization problem during the preparation. Even when the particles are oxidized during the preparation, the oxidized shells are removed through contact with sulfuric acid during the plating with nonmagnetic substance. These effects concur in order to greatly improve the magnetic characteristics of the produced hard magnetic material.

fter the plating, the highly magnetic particles are  
rtified against oxidization with the nonmagnetic shells  
nbracing them so that no oxidization should occur  
uring the subsequent compaction and sintering. Conse-  
iently, the high magnetic particles are free from en-  
rgement in deformation resistance which otherwise  
riously disables uniform deformation.

### EXAMPLE

This example is illustrative of the present invention 10  
it not to be construed as limiting the same.  
Carbonyl Fe powder particles of 99.5% purity, 5  $\mu\text{m}$   
verage diameter and 3 to 7  $\mu\text{m}$  grain size distribution  
as used for the highly magnetic substance. These car-  
bonyl Fe powder particles were plated with Cu by 15  
onelectrolytic plating so that the resultant Fe volume  
occupation ratio should be 59%. The plated Fe particles  
ere filled into a rubber casing of 100 mm. diameter and  
000 mm. length for hydrostatic compaction at 3,000  
 $\text{kg}/\text{cm}^2$  pressure. The compressed body was then sub-  
ected to sintering at 750° C. for 1 hour within  $\text{H}_2$  gass  
ivironment. Hydrostatic extrusion was applied to the  
ntered body at 13,000  $\text{kg}/\text{cm}^2$  pressure and 25:1 rate of  
ross-sectional reduction, which was followed by annealing  
at 650° C. for 30 min. Hydrostatic extrusion 25  
id annealing were alternately repeated until  
 $6.25 \times 10^4$  rate of cross-sectional reduction was finally  
ached. The produced hard magnetic material in-  
uded Fe fine grains having almost uniform diameter of  
out 20  $\mu\text{m}$ . As a result of magnetic characteristics 30  
easurement, it was confirmed that the hard magnetic  
aterial was 1.1 T in residual magnetic flux density,  
1,000 A/m in coercive force, and 47,000 AT/m in  
aximum magnetic energy product.

### COMPARATIVE EXAMPLE

An Fe rod of 99.99% purity and 2 mm. diameter was  
nfinied into a Cu cylinder of 2.8 mm. outer diameter  
nd 2 mm. inner diameter in order to form a composite  
ody. A plurality of such composite bodies were filled 40  
to a Cu cylindrical container of 150 mm. outer diameter  
nd 140 mm. inner diameter, which was then closed.  
ext, the container was subjected to hydrostatic extru-  
on at 100:1 rate of cross-sectional reduction, which  
as filled by annealing under process conditions same 45  
; that in the example of the present invention. Hydro-

static extrusion and annealing were repeated until  
 $1/1 \times 10^{10}$  rate of cross-sectional reduction was finally  
reached. The obtained hard magnetic material was 1.0  
T in residual magnetic flux density, 37,000 A/m in coercive  
force, and 18,000 AT/m in maximum magnetic  
energy product.

As is clear from the foregoing comparison, the process  
of the present invention assures stable production  
of hard magnetic material provided with highly im-  
proved magnetic characteristics at remarkably low pro-  
duction cost. In addition, it does not call for use of  
expensive metals such as Co, thereby lowering the ma-  
terial cost for production of such hard magnetic mate-  
rial.

We claim:

1. A process for producing hard magnetic material comprising plating powder particles of highly magnetic substance selected from the group consisting of Fe, Co, Ni and alloys thereof with nonmagnetic substance selected from the group consisting of Cu, Al, Sn, Pb, Zn and combination of these metals to form plated particles, said powder particles having a diameter from about 1 to about 1000 microns; compacting the plated particles; sintering the resulting compact; and subjecting the sintered compact to plastic deformation in a prescribed direction, thereby dispersing and orienting in said prescribed direction fine grains of said highly magnetic substance within a base of said nonmagnetic substance, each fine grain corresponding in size to the unit magnetic domain.
2. A process as claimed in claim 1 in which the combination of said highly magnetic and nonmag-  
netic substances is chosen from a group consisting  
of Fe with Cu at 10 to 85 volume occupation ratio  
of Fe, Fe with Pb at 10 to 85 volume occupation  
ratio of Fe, Fe with Sn at 10 to 80 volume occupa-  
tion ratio of Fe, and Fe with Zn at 10 to 80 volume  
occupation ratio of Fe.
3. A process as claimed in claim 1 in which  
said diameter of said powder particle is in a range  
from 5 to 150  $\mu\text{m}$ .
4. A process as claimed in claim 1, or 2, in which said  
plastic deformation is carried out by hydrostatic extru-  
sion.

\* \* \* \* \*